

## UNITED STATES PATENT OFFICE

2,361,582

NONSCUFFING WAX COATING  
COMPOSITION

Elmer Wade Adams, Hammond, and Frederick H. McLaren, Munster, Ind., assignors to Standard Oil Company, Chicago, Ill., a corporation of Indiana

No Drawing. Application February 27, 1942,  
Serial No. 432,628

9 Claims. (Cl. 196—149)

The present invention relates to improved wax compositions and methods of making them, and more particularly to such compositions suitable for waving paper sheets, paper cartons, and the like, to produce non-blocking and non-scuffing permanent coatings.

It is important for some uses that the wax coating have self-sealing properties. That is, when two pieces of wet-waxed paper are held in contact with heat applied for an instant, the wax films unite and the two sheets are bonded at that point. It is only when the wax is of high tensile strength that self-sealing properties are satisfactory.

To be commercially acceptable the wax coating, in addition to having a high tensile strength, must be free from scaling, peeling or scuffing and it must produce a non-blocking sheet. The sheets must not adhere when stacked and the coating must not strip off. For use on formed containers, which are coated by dipping the formed cardboard, such as milk caps, milk cartons and butter cartons, the odor, appearance, and particularly anti-scuffing of the coating are important. Therefore it is an object of this invention to produce an improved modified wax composition and coating of high tensile strength which is resistant to scaling and blocking.

The term "paraffin wax" as used herein defines the hard, non-ductile, crystalline wax comprising laminated plate-like crystals of paraffin, derived from paraffin base and mixed base type mineral oils. In recovering the paraffin wax, the crude oil is separated into a series of paraffin distillate fractions and the paraffin wax defined by well-known operations. For example, the wax-bearing distillate may be mixed with gas oil as a diluent to reduce the viscosity of the mass to facilitate pressing. This mixture may then be chilled in coolers at a definite chilling rate to produce crystals of optimum size for best rate of filtration. After the pressing is completed the slack wax is removed from the presses and reduced in a pipe still to remove the diluent. The reduced wax is then carried through the sweating operation. Sweating is a carefully controlled operation which involves drainage of the oil from the crystal interstices, fractional fusion, and the solubility effects of lower melting point waxes and oil. This operation is accomplished by slowly raising the temperature of the chilled crude scale wax at a uniform rate. A light clay percolation may be carried out on the refined wax as a final clean-up in the process. This percolation does

not affect the tensile strength but is principally for decolorization.

The physical properties of the paraffin wax are determined by the source of the crude oil from which the wax is prepared, the method of refining the paraffin wax, and the oil content of the resulting product. The paraffin wax used in our invention can be derived from Mid-Continent or Salt Creek crude and has a high tensile strength within the range of between about 250 and about 320 pounds per square inch or higher, a melting point within the range of between about 120° F. and about 140° F. and an oil content below about 0.3%, for example below about 0.1%. These waxes are white, brittle or non-ductile and granular.

Petrolatum wax may be obtained for similar crudes which have been stripped of their lighter fractions including the paraffin distillate. The stocks from which petrolatum waxes are made represent about a 25% bottoms of the original crude oils. The undistilled residue is refined by methods known to the art, as by diluting with an oil solvent and centrifuging, to produce a wax having a melting point within the range of between about 150° F. and 175° F., and ordinarily within the range of between about 155° F. and about 170° F., and an oil content of less than 6%. De-oiling may be accomplished by repeated solution, chilling and cold settling in naphtha, the oil being drawn off in the naphtha. Petrolatum waxes are smooth, ductile, tough materials, darker in color than the paraffin wax. The petrolatum wax is too ductile for dependable tensile strength tests but gives an apparent high tensile strength with necking down of the standard sample.

In carrying out the present invention to produce a wax composition of the character described, we may employ an improved wax composition comprising a low oil content, high tensile strength paraffin wax and a small percent of petrolatum wax to give a finished wax composition containing a maximum of about 0.2% oil which retains its initial high tensile strength and in addition is resistant to scuffing when applied as a coating. For example, such a composition may comprise 3% of 165° F. melting point petrolatum wax and 97% of 132° F. melting point paraffin wax of initially high tensile strength above about 250 pounds per square inch.

We have found that the non-scaling properties of a wax coating are affected by the crystal structure of the finished product. Paraffin wax of the prior art may be of low oil content and high ten-

sile strength but has a crystal form of laminated, even, flat, plate-like crystals. The coatings prepared from these high tensile strength, substantially oil-free straight waxes scuff and peel. Furthermore, we have found that although a coating of pure paraffin wax having a high tensile strength and low oil content may be satisfactory when first prepared, on aging there results a coating which scuffs and has the undesirable properties of the prior art. Sometimes coatings prepared from the paraffin wax are satisfactory for a short period due to the quick chilling effect of the waxing machine chill rolls. However, when used in wrappings and subjected to usual handling, crystal growth occurs and scuffing or "sloughing" becomes severe. This growth does not occur in coatings modified according to our invention.

Petrolatum wax differs from paraffin wax in crystal form, due primarily to difference in molecular weight. The addition of the small critical amounts of petrolatum wax to the high tensile strength paraffin wax modifies the crystal structure of the paraffin wax to produce jagged or curled interlocking crystals or aggregates with erose edges. The action of high melting petrolatum wax on crystal structure seems to be that of seeding due to the petrolatum wax chilling out first in the complex crystal system. Such change in crystal lattice imparts superior non-scaling properties to the composition without affecting the tensile strength.

A straight paraffin wax of very high tensile strength and good sealing properties does not assure a coating which is satisfactory from the standpoint of scaling in the rubbing test. The primary function of adding the petrolatum wax is to modify the crystal structure in such a manner that a coating prepared from the modified wax is non-scuffing. The highly refined unmodified paraffin waxes, whether of high or low tensile strength, both have large plate crystals. Thus, for example, two paraffin waxes having a tensile strength of 92 pounds per square inch and 304 pounds per square inch, respectively, each readily showed outlines of similar large plates when a 20% solution of the wax was viewed through a microscope wherein the crystals were magnified about 600 diameters. When the high tensile strength paraffin wax is modified by adding a small amount, for example 3% of 165° F. melting point petrolatum wax, the modified wax has substantially the same high tensile strength as the base material, i. e., about 304 pounds per square inch. However, the flat, even plate-like structure of the paraffin wax alone is completely gone and this wax composition is highly resistant to scuffing and is non-blocking.

Coatings prepared from the modified wax have substantially the same high tensile strength as the original paraffin waxes but in addition they are resistant to scuffing and blocking. The photomicrographs show that the cause of these excellent properties is the entirely different crystal structure of the wax blend than that of the highly refined paraffin wax without the small critical amount of added petrolatum wax. The addition of the small amounts of the petrolatum wax does not affect the already high tensile strength of the paraffin wax and the percent of oil is kept low in the finished coating to prevent blocking.

For example, a paper coated with a pure paraffin wax of 136° F. melting point and a high tensile strength within the range of between about 250 and 320 pounds per square inch, for example

312 pounds per square inch, and containing no more than 0.15% oil, for example 0.1%, scuffs and scales in the paper rubbing test. It is evident, therefore, that low oil content and high tensile strength alone are not indicative of a non-scuffing coating. However, the addition of from about 0.5% to about 3%, for example 0.75% to 1.5% of ductile petrolatum wax to the initially very high tensile strength paraffin wax greatly enhances the non-scuffing and non-blocking characteristics of this coating. The addition of corresponding amounts of petrolatum wax to low tensile strength paraffin waxes does not similarly enhance the non-scuffing characteristics of a coating although the tensile strength is improved.

Thus by adding a critical amount, for example about 3% of a petrolatum wax having a melting point of between about 155° F. and about 170° F., for example 165° F., and an oil content of less than 6% to unmodified very high tensile strength paraffin wax we obtain a new wax composition containing less than 0.2% oil and having substantially the same tensile strength as the unmodified paraffin wax. Such a wax composition has an entirely different crystalline structure than that of the initially high tensile strength paraffin wax. When applied as a coating the modified wax composition does not scuff or strip from the surface and is non-blocking.

Our invention is particularly useful in the preparation of wax-coated wrapping sheets and milk cartons, and may be applied by any of the conventional methods. For example, the wax composition when used on bread wrappers may first be applied in a light coat on one side before printing to prevent offset. After the ink has dried the sheet is given a final waxing on a machine in which the paper runs through a molten wax bath. This operation is followed by squeezing the hot sheet through rollers which, by regulation of the pressure, determine the thickness of the wax film. Following this the hot sheet is rapidly chilled by running it into a cool water bath or over a refrigerated roller. The final step in the manufacture of this type of wrapper is the cutting of the wide sheet into the proper size wrappers.

The stock may be ordinary sulphite pulp or it may be derived from various cellulose and regenerated cellulosic materials. To improve the wax coating and keep it on the surface of the coated materials, the stock may be wax-sized prior to the application of the new and improved wax composition. For example, petrolatum with or without the addition of other materials may be emulsified in the presence of a soap solution as the emulsifying agent to produce a size. However, the method of preparing an emulsion constitutes no part of the present invention. Such materials as paraffin wax, high melting point petrolatum bases, vegetable waxes, Montan wax, Ozokerite, resins or fatty materials may be incorporated in the paper-beating stage or any other suitable stage in advance of the formation of the sheet. Such a process aids in keeping the wax composition coating on the surface and results in better spreading of the coating, elimination of wax absorption, increased carton strength, and increased resistance to leakage.

Our new modified wax composition is very useful for coating wrapping sheets and the like, for example, those wrapping papers used on various food products. The high resistance of our improved wax composition coatings to scaling makes

them far superior to any composition of the prior art.

This application is a continuation-in-part of our copending application, Serial No. 333,686, filed May 6, 1940.

While our invention has been described with reference to particular examples, it is to be understood that the foregoing detailed description is given merely by way of illustration and that many modifications may be made therein without departing from the invention.

We claim:

1. An improved film-forming wax composition comprising a paraffin wax having an initial tensile strength of above about 250 pounds per square inch and normally forming a scuffing film and about 3% of a single wax-like addition agent consisting of a petroleum wax having a melting point at a temperature within the range of between about 155° F. and about 170° F. and an oil content of less than 6%, the said composition being further characterized by having a tensile strength substantially equal to that of the paraffin wax alone and by being resistant to scuffing and blocking when applied in a thin film.

2. An improved film-forming wax composition consisting of about 97% of a paraffin wax having a tensile strength of between about 250 and about 320 pounds per square inch and normally being subject to scuffing when in a thin film, and about 3% of a single wax-like addition agent consisting of a petrolatum wax having a melting point of about 165° F. and an oil content of less than 6% admixed with said high tensile strength paraffin wax, the wax composition being further characterized by containing a maximum of about 0.2% oil, by having a high tensile strength between about 250 and 350 pounds per square inch substantially equal to that of the paraffin wax alone and by being resistant to scuffing and blocking when applied in a thin film.

3. An improved wax-coating composition capable of being deposited in a non-scuffing film comprising between about 97% and about 99.5% of highly refined paraffin wax having a tensile strength above about 250 pounds per square inch, and between about 3% and about 0.5% of a single wax-like addition agent consisting of petroleum wax having a melting point above about 155° F. to about 170° F. and an oil content of less than 6%, the said wax-coating composition being resistant to scaling and blocking when applied in a thin film and having a tensile strength above about 250 pounds per square inch substantially equal to that of the paraffin wax alone.

4. An improved wax-coating composition capable of being deposited in a non-blocking and permanently non-scuffing film consisting of between about 0.5% and 3.0% of a petrolatum wax containing less than about 6% oil and having a melting point of about 165° F., and a paraffin wax having a high tensile strength above about 250 pounds per square inch and containing no more than about 0.15% oil, said composition having a tensile strength substantially equal to the tensile strength of the paraffin wax and having a net oil content of not more than 0.2%.

5. The method of rendering a paraffin wax resistant to scuffing, said wax normally having a high tensile strength of above about 250 pounds

per square inch and normally being subjected to scuffing when in a thin film, the step of permanently modifying the crystal structure of the paraffin wax by adding to said paraffin wax more than about 0.5% and less than about 5% of a single wax-like addition agent consisting of a ductile petrolatum wax having a melting point between 155° F. and about 170° F. and containing less than 6% oil whereby the surface coating characteristics of the paraffin wax are improved without substantially affecting the tensile strength thereof.

6. The method of rendering a paraffin wax resistant to scuffing, said wax normally having an initial tensile strength of between about 250 and 320 pounds per square inch and normally being subject to scuffing when in a thin film, the steps of permanently modifying the crystal structure of the paraffin wax by adding to said paraffin wax about 3% of a single wax-like addition agent consisting of a ductile petrolatum wax having a melting point between 155° F. and about 170° F. and containing less than 6% oil whereby the surface coating characteristics of the paraffin wax are improved without affecting the tensile strength thereof.

7. An improved wax coating composition consisting of at least about 97% of a paraffin wax having a tensile strength of between about 250 and about 320 pounds per square inch, said paraffin wax normally being subject to scuffing when applied in a thin film, and less than about 3% of a ductile petrolatum wax having a melting point of about 165° F. and an oil content of less than about 6%, the said coating composition being further characterized by having a tensile strength substantially within the range of the tensile strength of the paraffin wax alone and by being resistant to scuffing and blocking when applied in a thin film.

8. An improved wax coating composition free of polar wax-like substances and which is resistant to scuffing when applied in a thin film, said composition comprising essentially an admixture of paraffin wax normally having an initial tensile strength above about 250 pounds per square inch and normally forming a coating which scuffs and more than about 0.5% and less than about 5% of petrolatum wax having a melting point within the range of between about 155° F. and about 170° F. and an oil content of less than 6%, the tensile strength properties of said paraffin wax being substantially unaltered and the resistance to scuffing being substantially increased by the blending of the said petrolatum wax therewith.

9. An improved wax composition adapted to produce a thin film which is resistant to scuffing, said composition comprising an admixture of between about 0.5% and about 3.0% of a wax consisting a ductile petrolatum wax containing not more than about 6% oil and having a melting point within the range of between about 155° F. and about 170° F. and a base wax consisting of a paraffin wax which is characterized by having an initial high tensile strength of above about 250 pounds per square inch which tensile strength is substantially unchanged with an increase in the resistance to scuffing.

ELMER WADE ADAMS.  
FREDERICK H. MACLAREN.